

## UNITED STATES PATENT OFFICE

2,610,133

## PROCESSES OF BRIGHTENING AND PASSIVATING CADMIUM AND ZINC

Francis X. Thomson, Delaware Township, Camden County, N. J., assignor to Radio Corporation of America, a corporation of Delaware

No Drawing. Application October 26, 1949,  
Serial No. 123,798

7 Claims. (Cl. 148—6.21)

1

This invention relates to processes of brightening and passivating metallic surfaces. More particularly, the invention relates to processes of treating surfaces of cadmium, zinc, or alloys of these two metals.

In order to prevent rusting of objects made of iron or steel, and at the same time, to enhance their appearance, it is common practice to electroplate the objects with thin coatings of other metals more resistant to atmospheric corrosion. Among the metals commonly used for this purpose are cadmium and zinc. However, it is a characteristic of cadmium and zinc that freshly electrodeposited surfaces of these two metals quickly lose much of their luster, due to the formation of thin surface films of oxides, as a result of exposure to air.

In order to restore the brightness of surface coatings of cadmium and zinc, various methods have been used with more or less success. In most cases, however, brightness of the coating gradually decreases with age and, eventually, the original luster completely disappears. One of the methods previously used to brighten the surfaces of electrodeposited cadmium or zinc has been to dip the plated article in a dilute solution of nitric acid. This has the disadvantage, however, of making the surface more susceptible to atmospheric corrosion than an untreated surface. The use of various strong oxidizing acids as brightening agents is also well known. Although the surfaces thus treated resist ordinary atmospheric corrosion, these agents have various disadvantages in that they are not free rinsing, they are usually expensive, and they dissolve a considerable amount of cadmium or zinc from the plated article.

The process of the present invention has none of the above mentioned disadvantages and, on the other hand, is economical and simple to operate. Furthermore, the process can be used satisfactorily in automatic processing machines.

In general, the process comprises rinsing the plated part, dipping in dilute nitric acid, and then dipping in a solution of an alkali metal dichromate preferably containing an organic wetting agent. The treated part is then rinsed in water and dried.

One object of the invention is to provide an improved method of brightening and passivating a surface of substantially pure cadmium or zinc.

Another object of the invention is to provide an improved method of brightening and passivating a surface of electrodeposited cadmium or zinc.

Another object of the invention is to provide

2

an improved method of rendering a surface of substantially pure cadmium or zinc or alloys of the two metals resistant to the effects of atmospheric corrosion.

5 A further object of the invention is to provide an improved method of brightening and passivating a surface of substantially pure cadmium or zinc or of cadmium-zinc alloys without dissolving any appreciable quantities of the metal.

10 Still another object of the invention is to provide an improved process of brightening and passivating a surface of substantially pure cadmium or zinc in which the results are long lasting.

15 Other objects and advantages will be more apparent and the invention will be better understood from the further description which follows:

20

## Example

A cadmium plated part is, first, thoroughly rinsed in cold running water in order to remove all traces of the plating bath. The rinsed part is then dipped in a bath of 0.5% nitric acid for 20-30 seconds. The nitric acid bath consists essentially of a dilute, aqueous solution of the acid with the ingredients being present in a ratio of 0.5 cc. concentrated nitric acid in 100 cc. of solution. The article is then removed from this solution and, without rinsing off the solution clinging to the surface, is dipped for 20-30 seconds in a bath consisting essentially of 3 ounces of potassium dichromate and 2 ounces of a wetting agent per gallon of water. Any other alkali metal dichromate; for example, sodium dichromate, may be used and also any organic wetting agent which can be dissolved in the solution. Examples of suitable wetting agents are the well known alkyl-aryl polyether alcohols such as Triton NE (Rohm and Haas), sodium aryl alkyl sulfonate (nacconol NR, Allied Chemical and Dye Corporation), polyethylene glycol tertiary-dodecylthioether, and dodecyl toluene sodium sulfonate. The article is then removed from the bath, rinsed in running water maintained at about 190-210° F. and dried in hot air.

Once started, the process should be carried through to completion for best results. That is, the article should not be permitted to stand for any appreciable time between successive steps in the process. The concentrations of ingredients in the treating baths may be varied somewhat although the concentrations given in the example are preferred. In the first bath, the nitric acid concentration may vary between about 0.1% and

3% by volume. In the second bath, the dichromate may be present within a range of about 1-6 ounces per gallon of water and the wetting agent may be present within the range of about 1-8 ounces per gallon of water.

Although the particular wetting agent used is not critical except that one must be used which is compatible with the rest of the constituents of the treating bath, it is necessary that a wetting agent be used if good results are to be obtained. Without a wetting agent, the dichromate solution film tends to be discontinuous. This leads to early deterioration of the treated surface as well as non-uniform characteristics. When a wetting agent is included, the dichromate solution wets the metal surface uniformly.

The cadmium or zinc surface which is treated should be substantially pure metal of either one of the two metals or of any alloy of the two. Substantially pure surfaces are obtained by electrodeposition, chemical deposition, or vapor deposition in vacuo. Ordinary cast metal is usually not sufficiently pure for good results to be obtained and is not intended to be used with the present process.

Although a 20-30 second dip in dilute nitric acid is preferred, as stated in the example, dips of 10-40 seconds are almost as good. If the immersion time is longer than about 40 seconds, metal will begin to dissolve from the surface in appreciable amounts although the quality of the resulting product will not be diminished to any extent. The maximum immersion time is thus not critical except from the standpoint of wasting metal. The 20-30 second immersion in the second bath containing the dichromate and the wetting agent is even less critical although this time range is preferred. Longer times than 30 seconds produce no further improvement and are merely a waste of time.

The final rinsing step may take place in cold water, if desired. Warm water is used to aid rapid drying and rapid drying is preferred to avoid any tendency toward staining of the surface. This is also the reason why drying in hot air is preferred.

There has thus been described an improved process of brightening and passivating surfaces of substantially pure cadmium or zinc or alloys of the two metals. Treating with dilute nitric acid alone is much less satisfactory and it was also found that a single bath containing both the nitric acid and the dichromate did not produce the improved results. Although previous cleaning methods are known utilizing baths containing sulfuric acid and potassium dichromate,

this type of bath likewise will not produce the excellent results of the present method on cadmium or zinc surfaces.

I claim as my invention:

1. A process of brightening and passivating a metallic surface of at least one substantially pure metal from the class consisting of cadmium and zinc, comprising treating said surface with an aqueous solution of nitric acid in which the acid concentration is about 0.1 to 3% by volume, then treating said surface with an aqueous solution consisting essentially of about 1 to 6 ounces of an alkali dichromate salt and about 1 to 8 ounces of a wetting agent per gallon of water, rinsing the treated surface, and drying, said process being carried out without permitting the article being treated to stand for any appreciable time between successive steps.
2. A process according to claim 1 in which said surface is an electrodeposited layer of cadmium.
3. A process according to claim 1 in which said surface is an electrodeposited layer of zinc.
4. A process according to claim 1 in which the nitric acid concentration is 0.5% by volume, the alkali metal dichromate is potassium dichromate present in the amount of 3 ounces per gallon and the wetting agent is dodecyl toluene sodium sulfonate present in the amount of 2 ounces per gallon.
5. A process according to claim 1 in which the surface is immersed in said nitric acid solution for from 20 to 30 seconds and then immersed in the solution containing said dichromate and said wetting agent for from 20-30 seconds.
6. A process according to claim 1 in which the final rinsing treatment is carried out with water at a temperature of 190°-210° F.
7. A process according to claim 6 in which the finally rinsed surface is dried in hot air.

FRANCIS X. THOMSON

#### REFERENCES CITED

The following references are of record in the file of this patent:

#### UNITED STATES PATENTS

| Number    | Name              | Date          |
|-----------|-------------------|---------------|
| 2,035,380 | Wilhelm           | Mar. 24, 1936 |
| 2,186,579 | Dubpernell et al. | Jan. 9, 1940  |
| 2,446,060 | Pray et al.       | July 27, 1948 |
| 2,465,247 | McBride           | Mar. 22, 1949 |
| 2,477,810 | McLean et al.     | July 26, 1949 |
| 2,479,423 | Snyder            | Aug. 16, 1949 |

#### OTHER REFERENCES

Iron Age, July 26, 1945, pages 61 and 143.